

May 8, 1945.

P. P. ALEXANDER

2,375,200

## PURIFICATION OF BARIUM

Original Filed March 5, 1943



INVENTOR  
*PETER P. ALEXANDER*

BY

BY  
Frances Davis, Mason & Edmunds  
ATTORNEYS

## UNITED STATES PATENT OFFICE

2,375,200

## PURIFICATION OF BARIUM

Peter P. Alexander, Marblehead, Mass., assignor  
to Metal Hydrides Incorporated, Beverly, Mass.,  
a corporation of Massachusetts

Original application March 5, 1943, Serial No.  
478,095. Divided and this application April 26,  
1944, Serial No. 532,736

20 Claims. (Cl. 75—67)

This invention relates to the purification of barium contaminated with metal impurities having a lower boiling point, and has for its object more particularly certain improvements in the method of purifying barium contaminated with alkali metal impurities, such as sodium and potassium.

Barium metal is usually made by subjecting fused barium chloride to electrolysis. Since the salts of the alkali metals, sodium and potassium, are usually present in the barium chloride, the resulting barium metal is usually contaminated with a small amount of alkali metal, as well as of the barium chloride itself. To purify the barium metal, it has been proposed to subject it to distillation in a closed retort that has been evacuated to remove objectionable air. The distilled barium is permitted to condense in a cooler part of the retort, usually in the form of a more or less spongy deposit, while the alkali metal impurities condense in a still cooler part of the retort. After cooling the retort, air is admitted, the retort is opened and the condensed barium is removed. The resulting product is so reactive that it frequently oxidizes rapidly on the surface and produces heat in sufficient amount to ignite the whole mass, with the result that fires are quite common. This objectionable result is all the more apt to occur because of the presence of the more highly reactive sodium and potassium. The small deposits of sodium and potassium are so reactive that they almost invariably catch fire when the retort is opened and they come in contact with the oxygen of air.

As a result of my investigations, I have discovered that these disadvantages may be overcome for the most part. The alkali metals, sodium and potassium, may be segregated from the barium metal in a form to make them non-inflammable on exposure to the oxidizing influence of air. The barium metal may be separately collected and it may at the same time be substantially freed of its chloride.

In accordance with the invention, the barium metal is heated in the absence of air to a temperature sufficiently high to distill the alkali metal impurity or impurities. The alkali metal vapor is selectively oxidized by bringing it in reactive contact with a refractory oxide, such as titanium oxide, zirconium oxide and chromium oxide, and the resulting oxidized alkali metal impurity is collected as a solid separate from the barium metal to be purified. The barium metal itself is advantageously distilled and condensed separate from the oxidized alkali metal impurities.

These and other features of the invention may be better understood by referring to the accompanying drawing, taken in conjunction with the following description, in which:

Fig. 1 is a diagrammatic representation, being a side elevation in section, of an apparatus with which the method of the invention may be practiced; and

Fig. 2 is a horizontal section on the line 2—2 of Fig. 1.

The apparatus shown comprises an outer retort 10 supported within a heating furnace 11, the retort being held in position by means of two or more supports 12 resting on top of the heating furnace. The retort preferably consists of heat-resistant steel. It is provided with a removable cover 13 having attached thereto a vertical pipe 14 and lateral valved branches 15 and 16, connectible with a source of vacuum, and air, respectively. A removable inner retort 20, having an open top, rests within the outer retort. A removable tray 21 rests over the open top of the retort, being supported thereon by means of three or more lugs 22 extending over the wall of the inner retort. The heating furnace 11 consists essentially of a rectangular chamber 23 having a refractory bottom 24, side and end walls 25, and a top 26 having an opening of a size adapted to receive the outer retort. An expanding opening 27 is provided at or near a lower corner of one of the side walls of the chamber, for the introduction of heating gases into the chamber. A similar opening 28 is preferably provided at or near an opposite corner, as a spare or auxiliary means for introducing heating, or cooling, gases into the chamber. When not in use, the opening 28 is closed. A flue opening 29 extends through the same wall as the opening 27, preferably at a higher level, so that heating gases passed into the chamber through the opening 27 tend to pass around the retort before leaving the chamber through the flue opening 29.

The apparatus may be used as follows: A charge of barium, for example, contaminated with sodium, potassium, and barium chloride, is placed in the bottom of the inner retort 20. The inner retort is then placed in the outer retort 10. A layer of titanium oxide 30 is placed in the tray 21, which is in turn placed across the open top of the inner retort. The removable cover 13 is placed on the outer retort 10 and locked thereon to provide a sealed joint. The lateral branch 15 is then connected to a source of vacuum. With the valve of this lateral branch open, and the valve of the other lateral branch 16 closed, the

outer and inner retorts are placed under vacuum to remove objectionable air.

Heating gases are passed through opening 27 into the heating chamber, where they circulate almost completely around the retort and then pass through the flue opening 29 to the outside atmosphere. As the lower portion of the outer retort 10 is heated, the lower portion of the inner retort 20 is also heated. As the temperature rises, a point is reached where the sodium and potassium present in the barium are distilled. The resulting sodium and potassium vapors rise to the upper and cooler portion of the retort where they come in contact with the titanium oxide 30 in the tray 21. Due to their affinity for oxygen, the sodium and potassium are promptly oxidized and the titanium dioxide is reduced to titanium and a sub-oxide or titanium, according to reactions which may be indicated as follows:



As the temperature at the bottom of the inner retort continues to rise, a point is reached where the barium is distilled and its resulting vapor tends to condense and settle out against the wall of the inner retort immediately below the tray 16. Some barium vapor may of course rise sufficiently to come in contact with titanium dioxide in the tray and react with it in a manner similar to sodium or potassium vapor. The bulk of the distilled barium may, however, be separately condensed and collected, as shown. A residue consisting essentially of barium chloride, admixed perhaps with a small amount of sodium chloride or potassium chloride, or both, remains as a residue in the bottom of the inner retort.

The introduction of heating gases to the heating chamber is stopped and the retort is permitted to cool. The cooling operation may be accelerated by passing cooling air through the heating chamber, for example, through the opening 28, or by removing the outer retort and its contents from the heating chamber. After the retort has been suitably cooled, lateral branch 16 is opened to admit air to the interior of the retorts, after which the cover 13 is removed. The inner retort and tray are pulled out of the outer retort; the tray is removed, and the condensed barium is scraped off and separately recovered. The residues are advantageously removed by washing the inner retort with water.

It will be clear to those skilled in this art that the invention lends itself to numerous modifications. Instead of titanium oxide, other suitable refractory metallic oxides, such as zirconium oxide and chromium oxide, may be employed, either separately or admixed.

In the practice of the invention, advantage is taken of the relative boiling points of the metals. The boiling points of sodium and potassium are substantially below that of barium. The temperature of the barium is, therefore, gradually elevated to a point where the alkali metal impurity of lower boiling point is distilled. By heating its bottom, the retort is caused to yield a graduated temperature range, being hottest at its bottom and coolest at its top. Since the sodium and potassium have the lower boiling points, their vapors tend selectively to rise highest in the retort. Since the barium has the higher boiling point, its vapor tends not to rise

as high in the retort. The barium vapor meets a temperature environment conducive to condensation. In other words, the barium metal may be made to condense in an intermediate

5 section of the retort where the temperature is high enough to keep the alkali metal vapors in vapor form. The alkali metal vapors, on the other hand, tend to rise to a cooler portion of the retort, where they were heretofore condensed, 10 but where they are now converted into harmless compounds in accordance with the present invention.

This application is a division of my co-pending application Serial No. 478,095, filed March 5, 15 1943.

I claim:

1. In the method of purifying barium contaminated with an alkali metal impurity, the improvement which comprises heating the barium in the absence of air to a temperature at which the alkali metal impurity but not the barium is distilled, selectively oxidizing the resulting alkali metal impurity vapor in a zone removed from the main body of barium to be purified, and collecting the oxidized alkali metal impurity as a solid separate from the barium to be purified.

2. Method according to claim 1, in which the resulting vapor of the alkali metal impurity is selectively oxidized by bringing it into reactive contact with a refractory metal oxide in a zone removed from the main body of barium to be purified.

3. Method according to claim 1, in which the resulting vapor of the alkali metal impurity is selectively oxidized by bringing it into reactive contact with titanium oxide in a zone removed from the main body of barium to be purified.

4. Method according to claim 1, in which the resulting vapor of the alkali metal impurity is selectively oxidized by bringing it into reactive contact with zirconium oxide in a zone removed from the main body of barium to be purified.

5. Method according to claim 1, in which the resulting vapor of the alkali metal impurity is selectively oxidized by bringing it into reactive contact with chromium oxide in a zone removed from the main body of barium to be purified.

6. Method according to claim 1, in which the barium to be purified is also distilled, and condensing the resulting barium vapor as a solid separate from the oxidized alkali metal impurity in a zone intermediate that in which the alkali metal impurity is oxidized and that from which the main body of barium is distilled.

55 7. In the method of purifying barium contaminated with sodium as an impurity, the improvement which comprises heating the barium in the absence of air to a temperature sufficiently high to distill the sodium but not the barium, selectively oxidizing the resulting sodium vapor in a zone removed from the main body of barium to be purified, and collecting the oxidized sodium as a solid separate from the barium.

65 8. Method according to claim 7, in which the resulting sodium vapor is selectively oxidized by bringing it into reactive contact with a refractory metal oxide in a zone removed from the main body of barium to be purified.

9. Method according to claim 7, in which the resulting sodium vapor is selectively oxidized by bringing it into reactive contact with titanium oxide in a zone removed from the main body of barium to be purified.

70 10. Method according to claim 7, in which the resulting sodium vapor is selectively oxidized by

bringing it into reactive contact with zirconium oxide in a zone removed from the main body of barium to be purified.

11. Method according to claim 7, in which the resulting sodium vapor is selectively oxidized by bringing it into reactive contact with chromium oxide in a zone removed from the main body of barium to be purified.

12. Method according to claim 7, in which the barium to be purified is also distilled, and condensing the resulting barium vapor as a solid separate from the oxidized sodium impurity in a zone intermediate that in which the sodium impurity is oxidized and that from which the main body of barium is distilled.

13. In the method of purifying barium contaminated with potassium as an impurity, the improvement which comprises heating the barium in the absence of air to a temperature sufficiently high to distill the potassium but not the barium, selectively oxidizing the resulting potassium vapor in a zone removed from the main body of barium to be purified, and collecting the oxidized potassium as a solid separate from the barium.

14. Method according to claim 13, in which the resulting potassium vapor is selectively oxidized by bringing it into reactive contact with a refractory metal oxide in a zone removed from the main body of barium to be purified.

15. Method according to claim 13, in which the resulting potassium vapor is selectively oxidized by bringing it into reactive contact with titanium oxide in a zone removed from the main body of barium to be purified.

16. Method according to claim 13, in which the resulting potassium vapor is selectively oxidized by bringing it into reactive contact with zirconium oxide in a zone removed from the main body of barium to be purified.

17. Method according to claim 13, in which the

resulting potassium vapor is selectively oxidized by bringing it into reactive contact with chromium oxide in a zone removed from the main body of barium to be purified.

18. Method according to claim 13, in which the barium to be purified is also distilled, and condensing the resulting barium vapor as a solid separate from the oxidized potassium impurity in a zone intermediate that in which the potassium impurity is oxidized and that from which the main body of barium is distilled.

19. In the method of purifying barium contaminated with an alkali metal impurity, the improvement which comprises heating the barium in the absence of air to a temperature at which the alkali metal impurity but not the barium is distilled, selectively oxidizing the resulting alkali metal impurity vapor by bringing it into reactive contact with a refractory metal oxide in a zone removed from the main body of barium to be purified, and collecting the oxidized alkali metal impurity as a solid separate from the barium to be purified.

20. In the method of purifying barium contaminated with sodium as an impurity, the improvement which comprises heating the barium in the absence of air to a temperature sufficiently high to distill the sodium but not the barium, selectively oxidizing the resulting sodium vapor by bringing it into reactive contact with a refractory metal oxide in a zone removed from the main body of barium to be purified, collecting the oxidized sodium as a solid separate from the barium, distilling the barium, and condensing the resulting barium vapor as a solid separate from the oxidized sodium impurity in a zone intermediate that in which the sodium impurity is oxidized and that from which the main body of barium is distilled.

PETER P. ALEXANDER.